

## UNITED STATES PATENT OFFICE

2,167,064

## LUBRICANT

Melvin A. Dietrich, Wilmington, Del., assignor to  
 E. I. du Pont de Nemours & Company, Wilming-  
 ton, Del., a corporation of Delaware

No Drawing. Application June 2, 1936,  
 Serial No. 83,075

21 Claims. (Cl. 87—9)

This invention relates to lubricating oils and more particularly to a process for improving the viscosity-temperature relationships of lubricating oils.

5 The use of polymerized hydrocarbons and their hydrogenation products as well as hydrogenated rubber has been proposed. Patent 1,998,350 issued to Carl Wulff covers the addition of viscosity improving agents to lubricating oils, 10 which agents are selected from hydrocarbons having a molecular weight of more than 800, and from groups consisting of polymerization products of unsaturated hydrocarbons capable of forming polymeric homologous series together 15 with their products obtained by hydrogenation or isomerization. Polymers mentioned are those obtained from styrene, isobutylene, butadiene, hydrogenated rubber, cyclorubber, and hydrogenated cyclorubber. British Patent 379,717 is similar to the above U. S. patent. French Patent 760,861 delivered December 27, 1933, discloses the hydrogenation of lubricating oils and the addition to these oils of various polymeric agents free of oxygen for example hydrogenated rubber. 25 French Patent 762,289 delivered January 18, 1934, covers the addition to lubricating oils of polymeric hydrocarbon substances either by direct addition of the polymer or by adding the unsaturated hydrocarbon to the oils, followed by 30 polymerization. British Patent 422,471 accepted January 7, 1935, covers a process for the production of high quality lubricating oils which consists in treating the oils with liquefied hydrocarbons which are gaseous at ordinary temperatures, such as propane, to remove asphaltic material, followed by the addition of a synthetic hydrocarbon product of high molecular weight, soluble in the oil.

When the processes of the above patents are 40 followed, oils of improved viscosity are obtained but the agents employed have a pronounced thickening effect on the oils and act as viscosity improving agents solely by their ability to maintain viscosity at high temperatures. These materials must be applied to oils having an initial viscosity very materially lower than that of the desired product.

An object of the present invention is to improve upon the processes of the prior art as exemplified by the above patents. A further object is the production of improved lubricating oils by a process which will avoid a thickening action and permit the use of either initially high or low viscosity oils. A further object is to produce medium heavy lubricating oils of high vis-

cosity index from heavy oils. Still further objects are to provide new compositions of matter and to advance the art. Still other objects will appear hereinafter.

The above objects may be accomplished in accordance with my invention which comprises adding to a lubricating oil the combination of an oil soluble polymerized aliphatic hydrocarbon product having a molecular weight of at least 800 and a material capable of dissociating 5 aggregates of oil molecules which form in mineral oils as the temperature is lowered. The polymeric substances may be any of such substances disclosed in the patents hereinbefore referred to. However, I preferably employ hydrogenated rubber or polymeric products derived from cracked light ends of refinery gasoline, which products do not decompose appreciably on heating to a temperature of 200° C. for a 10 period of 5 minutes.

I have found that materials capable of dissociating aggregates of oil molecules are hydrogenated condensed ring compounds. Preferably, these compounds should be devoid of acidic substituents. Also, the substituents, if any, should 15 be devoid of elements other than carbon, hydrogen, oxygen and nitrogen. The most effective compounds appear to be hydrocarbon compounds consisting solely of carbon and hydrogen. Of these, decahydronaphthalene appears to be the 20 most satisfactory although other suitable compounds are tetrahydronaphthalene, hydrogenated anthracene, beta-naphthanone, hydrogenated alpha-naphthylamine, and the like.

The quantities of my compounds added to the 25 oil will be determined by the characteristics desired in the finished product and by the molecular weight of the polymeric agent. In general, however, the quantity of polymeric agent will not exceed 30% and preferably will lie between 0.2 30 per cent and 10 per cent by weight of the oil. In practice the quantity will generally range from about 0.3 per cent to about 5 per cent by weight of the oil. The quantity of the dissociating agent will usually not exceed 50 per cent. I preferably 35 use from about 5 to about 20 per cent by weight of the oil. In practice, the amount of dissociating agent will range from about 10 to about 20 per cent.

Preferably, the polymeric substance is dispersed in the dissociating agent and the resulting mixture is stirred into the oil while heating to 40 150° C. until complete homogeneity is obtained.

In order to more fully illustrate my invention, the preferred modes of carrying the same 45

into effect and the advantageous results to be obtained thereby, solutions were prepared as described in the preceding paragraph. The improvement in the quality of the oil was measured by determining the viscosity at 100° F. and 210° F. and then calculating the viscosity index according to the method described by Dean and Davis in Chem. and Met. Eng. 36, 618 (1929). This index serves as a measure of the flatness of the viscosity-temperature curve of an oil. With increasing values of the index, viscosity-temperature curves become flatter. Table I gives the results obtained on one oil.

Table I

| Material added to oil                                 | Saybolt Universal viscosity |            | Viscosity index |
|-------------------------------------------------------|-----------------------------|------------|-----------------|
|                                                       | 100° F.                     | 210° F.    |                 |
| None                                                  | Seconds 273                 | Seconds 48 | 63              |
| 2% hydrogenated rubber                                | 1080                        | 108        | 116             |
| 2% hydrogenated rubber+10% decahydronaphthalene       | 622                         | 85.5       | 127             |
| 2% hydrogenated rubber+20% decahydronaphthalene       | 450                         | 69         | 125             |
| 2% polymerized cracked gases                          | 1315                        | 138.5      | 124             |
| 2% polymerized cracked gases+10% decahydronaphthalene | 775                         | 108        | 133             |

Following the same procedure with another oil, the results in Table II were obtained.

Table II

| Material added to oil                                   | Saybolt Universal viscosity |              | Viscosity index |
|---------------------------------------------------------|-----------------------------|--------------|-----------------|
|                                                         | 100° F.                     | 210° F.      |                 |
| None                                                    | Seconds 329                 | Seconds 54.2 | 97              |
| 0.3% polymerized cracked gases                          | 411                         | 61           | 108             |
| 0.3% polymerized cracked gases+10% decahydronaphthalene | 260                         | 55           | 129             |

It will be noted that in each case a distinct improvement was obtained in the viscosity index of the oil by the use of the decahydronaphthalene-polymer combination over the use of the polymer alone. It will also be noted that the viscosity at both 100 and 210° F. is affected to a very much smaller extent by the use of the combination than by the use of the polymer itself.

The materials of my invention may be added separately to the oil, as hereinbefore described, or may be mixed with each other and subsequently added to the oil. In certain cases the desired effect may be secured by dissolving the raw materials in the oil followed by polymerization or by hydrogenation. For example, rubber and naphthalene could be dissolved in the oil and the mixture hydrogenated to produce an effect equivalent to the direct addition of corresponding amounts of hydrogenated rubber and decahydronaphthalene to the hydrogenated oil. Isobutylene or butadiene or other mixtures of olefines may be dissolved in the oil together with naphthalene and the mixture polymerized and then hydrogenated. Various other changes and modifications may be made in my invention without departing from the spirit thereof. Accordingly, my invention is to be limited solely by the appended claims construed as broadly as is permissible in view of the prior art.

I claim:

1. A composition of matter comprising a lubricating oil having incorporated therein about 0.2

to about 30% of a polymerized aliphatic hydrocarbon product having a molecular weight of at least 800 and from about 5 to about 50% of a hydrogenated condensed ring compound devoid of acidic substituents. 5

2. A composition of matter comprising a lubricating oil having incorporated therein about 0.2 to about 30% of a polymerized aliphatic hydrocarbon product having a molecular weight of at least 800 and from about 5 to about 50% of a 10 hydrogenated condensed ring compound devoid of acidic substituents and substituents containing elements other than carbon, hydrogen, oxygen and nitrogen.

3. A composition of matter comprising a lubricating oil having incorporated therein about 0.2 to about 30% of a polymerized aliphatic hydrocarbon product having a molecular weight of at least 800 and from about 5 to about 50% of a 20 hydrogenated condensed ring compound consisting of carbon and hydrogen. 15

4. A composition of matter comprising a lubricating oil having incorporated therein about 0.2 to about 30% of a polymerized aliphatic hydrocarbon product having a molecular weight of at least 800 and from about 5 to about 50% of an 25 unsubstituted hydrogenated condensed ring compound.

5. A composition of matter comprising a lubricating oil having incorporated therein about 0.2 to about 30% of a polymerized aliphatic hydrocarbon product having a molecular weight of at least 800 and from about 5 to about 50% of a 30 hydrogenated naphthalene.

6. A composition of matter comprising a lubricating oil having incorporated therein about 0.2 to about 30% of hydrogenated rubber and from about 5 to about 50% of a hydrogenated 35 condensed ring compound devoid of acidic substituents. 40

7. A composition of matter comprising a lubricating oil having incorporated therein about 0.2 to about 30% of hydrogenated rubber and from about 5 to about 50% of a hydrogenated 45 condensed ring compound consisting of carbon and hydrogen.

8. A composition of matter comprising a lubricating oil having incorporated therein about 0.2 to about 30% of hydrogenated rubber and from about 5 to about 50% of a hydrogenated 50 naphthalene.

9. A composition of matter comprising a hydrocarbon oil having incorporated therein about 0.2 to about 30% of a polymerized aliphatic hydrocarbon product having a molecular weight of at 55 least 800 and from about 5 to about 50% of a hydrogenated condensed ring compound devoid of acidic substituents.

10. A composition of matter comprising a hydrocarbon oil having incorporated therein about 0.2 to about 30% of a polymerized aliphatic hydrocarbon product having a molecular weight of at least 800 and from about 5 to about 50% of a 60 hydrogenated condensed ring compound consisting of carbon and hydrogen. 65

11. A composition of matter comprising a hydrocarbon oil having incorporated therein about 0.2 to about 30% of a polymerized aliphatic hydrocarbon product having a molecular weight of at least 800 and from about 5 to about 50% of a 70 hydrogenated naphthalene.

12. A composition of matter comprising a hydrocarbon oil having incorporated therein about 0.2 to about 30% of hydrogenated rubber and from about 5 to about 50% of a hydrogenated 75

condensed ring compound consisting of carbon and hydrogen.

13. A composition of matter comprising a hydrocarbon oil having incorporated therein about 5 0.2 to about 30% of hydrogenated rubber and from about 5 to about 50% of a hydrogenated naphthalene.

14. A composition of matter comprising a lubricating oil having incorporated therein about 10 0.2 to about 30% of a polymerized aliphatic hydrocarbon product having a molecular weight of at least 800 and from about 5 to about 50% of decahydronaphthalene.

15. A composition of matter comprising a hydrocarbon oil having incorporated therein about 15 0.2 to about 30% of a hydrogenated rubber and from about 5 to about 50% of decahydronaphthalene.

16. A composition of matter comprising a lubricating oil having incorporated therein about 20 0.2 to about 30% of polymerized cracked gases having a molecular weight of at least 800 and from about 5 to about 50% of a hydrogenated condensed ring compound devoid of acidic 25 constituents.

17. A composition of matter comprising a hydrocarbon oil having incorporated therein about 0.2 to about 30% of polymerized cracked gases having a molecular weight of at least 800 and

from about 5 to about 50% of a hydrogenated condensed ring compound devoid of acidic substituents.

18. A composition of matter comprising a hydrocarbon oil having incorporated therein about 5 0.2 to about 30% of polymerized cracked gases having a molecular weight of at least 800 and from about 5 to about 50% of a hydrogenated condensed ring compound consisting of carbon and hydrogen.

19. A composition of matter comprising a hydrocarbon oil having incorporated therein about 10 0.2 to about 30% of polymerized cracked gases having a molecular weight of at least 800 and from about 5 to about 50% of a hydrogenated 15 naphthalene.

20. A composition of matter comprising a lubricating oil having incorporated therein about 0.2 to about 30% of polymerized cracked gases 20 having a molecular weight of at least 800 and from about 5 to about 50% of decahydronaphthalene.

21. A composition of matter comprising a hydrocarbon oil having incorporated therein about 0.2 to about 30% of polymerized cracked gases 25 having a molecular weight of at least 800 and from about 5 to about 50% of decahydronaphthalene.

MELVIN A. DIETRICH.